

## UNITED STATES PATENT OFFICE

2,658,866

## ELECTRODEPOSITION OF TIN-NICKEL ALLOY

Norman Parkinson, Hayes, England, assignor to  
John Ireland, Middlesex, EnglandNo Drawing. Application May 9, 1950,  
Serial No. 161,017Claims priority, application Great Britain  
November 22, 1949

1 Claim. (Cl. 204—43)

1

This invention relates to the electrodeposition of tin-nickel alloy.

The electrodeposition of tin and nickel separately is well known as is also the principle of using small quantities of a second metallic ion to improve the smoothness of the deposit of the primary metal. Thus one particular proposal that has been made is to use from 2 to 10 g./l. of a nickel salt to improve the tin coating deposited from a bath containing stannous chloride and alkali fluoride but to obtain satisfactory deposits from this bath it is essential that it contains one or more of the organic addition agents used in the electro-plating industry for improving the smoothness of deposits.

According to the present invention I electrodeposit tin-nickel alloy coatings containing not more than 90% nor less than 50% of tin from an aqueous solution of appropriate salts of tin and nickel containing the respective metals in proportions between 2:1 and 1:7.

The electrolyte must contain tin and nickel cations and may contain the cations of an alkali metal including ammonium. The anions may be chlorides alone, or chlorides and fluorides, or chlorides sulphates and fluorides, or fluorides alone.

An important feature of the baths used in accordance with the present invention is that they produce satisfactory smooth deposits in the absence of organic addition agents.

The tin and nickel cations may be replenished by using anodes of an appropriate tin-nickel alloy. Alternatively separate tin anodes and nickel anodes may be used. In the latter case replenishment may be effected either by passing the total current through each anode successively for an appropriate time or by using the tin and nickel anodes simultaneously and apportioning the current through them appropriately.

For some purposes it may be convenient to use either tin anodes or nickel anodes and to supply the other metallic cation by adding to the bath suitable salts.

Further features of the invention will be apparent from the examples given hereafter of baths that I have found to give satisfactory results at the temperature and with the current density shown. Approximate composition of the alloy coating obtained is also shown.

2

Example I

|                                       | G./l. |
|---------------------------------------|-------|
| SnCl <sub>2</sub> , 2H <sub>2</sub> O | 100   |
| NiCl <sub>2</sub> , 6H <sub>2</sub> O | 400   |
| NaF                                   | 55    |
| NH <sub>4</sub> HF <sub>2</sub>       | 70    |

Temperature 65° C., 27 amps./sq. ft. Coating Sn 55%, Ni 45%.

10

Example II

|                                       | G./l. |
|---------------------------------------|-------|
| SnCl <sub>2</sub> , 2H <sub>2</sub> O | 100   |
| NiF <sub>2</sub>                      | 75    |
| NiCl <sub>2</sub> , 6H <sub>2</sub> O | 325   |
| KCl                                   | 100   |

Temperature 65° C., 20 amps./sq. ft. Coating Sn 70%, Ni 30%.

20

Example III

|                                       | G./l. |
|---------------------------------------|-------|
| SnF <sub>2</sub>                      | 40    |
| NaF                                   | 75    |
| NiCl <sub>2</sub> , 6H <sub>2</sub> O | 200   |

Temperature 65° C., 27 amps./sq. ft. Coating Sn 80%, Ni 20%.

25

Example IV

|                                       | G./l. |
|---------------------------------------|-------|
| SnCl <sub>2</sub> , 2H <sub>2</sub> O | 50    |
| NaF                                   | 30    |
| NH <sub>4</sub> HF <sub>2</sub>       | 30    |
| NiCl <sub>2</sub> , 6H <sub>2</sub> O | 60    |

Temperature 65° C., 24 amps./sq. ft. Coating Sn 82%, Ni 18%.

30

Example V

|                                                              | G./l. |
|--------------------------------------------------------------|-------|
| SnCl <sub>2</sub> (anhydrous)                                | 20    |
| NiCl <sub>2</sub> , 6H <sub>2</sub> O                        | 300   |
| Temperature 65° C., 10 amps./sq. ft. Coating Sn 67%, Ni 33%. |       |

It is to be understood, however, that the foregoing examples are given purely by way of illustration to describe the nature of the invention and not to limit its scope, and we may vary the actual ingredients of the baths and the proportions of such ingredients as also the operating temperature and current density depending upon

35

any practical requirements that may have to be fulfilled.

I claim:

A process which comprises electrodepositing tin-nickel alloy coatings from an aqueous solution bath constituted as follows:

|                                       |     |       |           |
|---------------------------------------|-----|-------|-----------|
| SnCl <sub>2</sub> , 2H <sub>2</sub> O | 100 | G./l. | 1,404,156 |
| NiCl <sub>2</sub> , 6H <sub>2</sub> O | 400 |       | 2,085,543 |
| NaF                                   | 55  |       | 2,119,304 |
| NH <sub>4</sub> HF <sub>2</sub>       | 70  | 10    | 2,183,384 |
|                                       |     |       | 2,381,778 |

NORMAN PARKINSON.

References Cited in the file of this patent

UNITED STATES PATENTS

| Number     | Name               | Date          |
|------------|--------------------|---------------|
| Re. 11,624 | Alexander          | Aug. 3, 1897  |
| 1,404,156  | Marino             | Jan. 17, 1922 |
| 2,085,543  | Oplinger           | June 29, 1937 |
| 2,119,304  | Viers et al.       | May 31, 1938  |
| 2,183,384  | Viers et al.       | Dec. 12, 1939 |
| 2,381,778  | Schoonmaker et al. | Aug. 7, 1945  |